

1

3,575,686

## TREATMENT OF TEXTILES

John William Case, Norman Frederick Crowder, and Wilfred Arthur Stephen White, Runcorn, England, assignors to Imperial Chemical Industries Limited, London, England

No Drawing. Continuation-in-part of application Ser. No. 549,498, May 12, 1966. This application Oct. 14, 1966, Ser. No. 586,663

Claims priority, application Great Britain, June 24, 1965,

21,905/65

Int. Cl. D06I 1/02

U.S. Cl. 8—142

6 Claims

## ABSTRACT OF THE DISCLOSURE

There is provided an improvement in the process whereby textile materials are solvent scoured. The solvent is flashed off and thereafter the textile material is finished or dyed. The improvement resides in applying the finish or dyestuff in the flash-off stage of the known process.

This application is a continuation-in-part of copending application Ser. No. 549,498, filed on May 12, 1966, now U.S. Pat. No. 3,476,504.

This invention relates to a process for the treatment of textile materials and more particularly to process improvements or modifications which can be used in conjunction with the scouring of textile materials with organic solvents.

It is known, for example in U.K. specifications Nos. 812,984 and 916,338 to treat textile materials with an organic solvent, particularly a chlorinated hydrocarbon solvent, in order to clean them. This procedure is sometimes termed a solvent scouring treatment. In such a process the textile material is passed through a bath of organic solvent, under conditions which enable contamination to be removed from the textile materials, and then the treated textile material laden with solvents is passed through an apparatus in which the solvent is evaporated and recovered. This final stage commonly termed the "flash-off stage," may be carried out using hot water or steam.

We have now found that this procedure is especially useful when carried out in conjunction with dyeing the material while it is in an open and absorbent condition by including a dyestuff in the water used in the flash-off system. This procedure can be modified so as to apply a finishing agent to the material.

According to our invention we provide a process for the treatment of a textile material which comprises scouring the textile material with an organic solvent, removing the solvent from the textile material in an aqueous flash-off stage and application of a dyestuff or finishing agent to the textile material in the aqueous flash-off stage.

When steam is used it is usual to pass the textile material from the solvent bath through squeeze rollers to remove excess solvent, and then through an aqueous flash-off stage which comprises a space in which the textile material is contacted with steam and a water seal through which the textile material leaves the apparatus. In such a case the dyestuff or finishing agent will be incorporated in the water seal.

When hot water and not steam is used in the "flash-off stage" it is usual for the textile material to pass from the solvent bath through squeeze rollers to remove excess solvent and then directly into a bath of water held at a sufficiently high temperature to "flash-off" the solvent. In such a case the hot water "flash-off" bath will contain the dyestuff or finishing agent.

2

Our process is particularly convenient when the textile material to be treated contains only solvent-soluble textile assistants, for example assistants (such as sizes), which have been applied to the textile fibres from solution in an organic solvent as is more fully described in our copending U.K. application No. 21,906/65.

By using, prior to the solvent scouring stage, textile assistants which are entirely soluble in the organic solvent we find that the solvent scouring stage can remove practically all contamination from the textile material and leave it in such a condition that, after the adherent organic solvent is removed, it is thoroughly clean and absorbent and in an excellent condition for dyeing.

When the textile assistants used in the weaving of

15 the textile material are not entirely solvent-soluble, there may be a tendency for any residues remaining on the cloth after the solvent scouring stage to interfere slightly with the efficiency of the stage in which the dye or finishing agent is applied, though in many cases this may 20 not be of more importance than slightly decreasing the efficiency of finishing agent or dyestuff usage. It is however generally desirable to remove as much contamination as possible before the textile is passed to the stage at which the dye or finishing agent is applied, and if necessary an aqueous desizing step may precede the solvent scouring step. A preliminary aqueous desizing step is particularly advantageous when a starch, cellulose ether or similar size has been used on a fibre, for example on cellulose fibre such as cotton or rayon.

30 The solvents and techniques which can be used for the solvent scouring stage may be in particular any of those described more fully in U.K. specifications Nos. 812,984; 916,338; 747,481; 749,705; 812,893; 844,943; 825,402; 1,042,398 and patent application No. 9,975/65. Thus the

35 solvent may be in particular trichloroethylene, perchloroethylene, 1,1,2-trichloro-1,2,2-trifluoroethane or mixtures thereof. The choice of solvent to be used depends very much upon the particular textile material concerned and the solvent is best chosen so that its solvent properties

40 and boiling point are such that its use will not adversely affect the textile material. In particular, it may be appropriate to use a low-boiling solvent, for example, 1,1,2-trichloro-1,2,2-trifluoroethane, in the case of textile materials which are particularly sensitive to heat or solvent action.

45 During the solvent "flash-off" solvent or an azeotrope of the solvent and water is vigorously evaporated thus leaving the textile material in an open and highly absorbent state and we believe that one of the advantages of 50 our process lies in the application of the dyestuff or finishing agent to the material while it is in such a highly absorbent state, thus giving a high rate of uptake and a high and even penetration of dyestuff or finishing agent.

55 The application of a dyestuff may involve the use of any of the conventional dyestuffs, dyeing assistants and auxiliary products known in the art, and these may be selected appropriately to the textile material concerned. Suitable dyestuffs include water-soluble, water-dispersible and reactive dyes and suitable finishing agents include brightening and softening agents and fluorescent whiteners. The temperature of the dye bath, when the textile material is dyed in a hot-water flash off, should be sufficiently high to ensure the rapid removal of the solvent (a minimum temperature of 86° C. and 73° C. is required 60 for perchloroethylene and trichloroethylene respectively). When the textile is dyed in a water seal after contact with steam the temperature of the dye bath need not necessarily be so high. Times of residence in the solvent-scouring bath, the steam treatment chamber and/or the bath in which the dye or finishing agent are applied will 65 vary with the textile material to be treated, the solvent

70

used and the type of dye or finishing agent to be applied. Suitable times may be found very easily by simple experiment, but in general we have found that times of from 10 to 60 seconds in the solvent bath, and from 10 to 30 seconds in a steam flash-off chamber (if used) are suitable. The time of residence in the bath in which the dyestuff or finishing agent is applied to the textile material will vary with the method of application, for example times of from 2 to 60 seconds are suitable for dyestuffs or finishing agents which are simply applied to the textile material in the bath and are then set on the material at a later stage, but times of up to about 5 minutes may be necessary if transfer of dyestuff or finishing agent onto the material occurs only in the bath and there is no subsequent setting stage. The concentration of dyestuff or finishing agent and the general conditions under which it is applied will be those well known in the art or will be slightly modified in obvious ways to suit the particular conditions pertaining.

The invention is illustrated but in no way limited by reference to the following examples in which the parts are by weight.

#### EXAMPLE 1

100 parts of (a) a plain weave cotton fabric or (b) a heavy cotton canvas or (c) a medium spun viscose rayon were separately immersed in 5000 parts of boiling trichloroethylene for a period of 30 seconds. The fabric was removed from the trichloroethylene, squeezed between rollers to a total weight of 250 parts and entered directly into 5000 parts of a boiling, aqueous dyebath containing 50 parts of those dyes recorded in the Colour Index as (a) Direct Red 1 (CI 22310) (b) Direct Blue 86 (CT 74180) (c) Direct Blue 76 (CI 22410). After 30 seconds immersion the fabric was removed, squeezed through rollers to a total weight of 200 parts and dried in hot air. The fabric was in each of the nine possible combinations of the three individual fabrics with the three individual dyestuffs dyed to a level, well penetrated shade.

#### EXAMPLE 2

100 parts of (a) Botany wool serge fabric (b) wool felt fabric, (c) spun nylon 66 fabric, (d) a fabric woven from nylon 6 filament were separately immersed in 5000 parts of boiling trichloroethylene for a period of 30 seconds. 45

The fabric was removed from the trichloroethylene, squeezed between rollers to a total weight of 240 parts and entered directly into 5000 parts of a boiling, aqueous dyebath containing 50 parts of a dye recorded in the Colour Index as Acid Blue 138 (CI 62075). After 30 seconds immersion the fabric was removed, squeezed through rollers to a total weight of 200 parts and dried in hot air. In each case the fabric was dyed to a level, well penetrated blue shade.

What we claim is:

1. In a process for the treatment of a textile material by scouring the textile material with an organic solvent, removing the solvent from the textile material in an aqueous flash-off stage and applying a member selected from the group consisting of a dyestuff and finishing agent to the textile material the improvement comprising applying the said member in the flash-off stage.
2. Process as claimed in claim 1 wherein the said member is applied to the textile material in a hot water flash-off bath.
3. Process as claimed in claim 1 wherein the textile material is subjected to an aqueous desizing step before it is scoured with the organic solvent.
4. Process as claimed in claim 1 wherein the textile remains in a solvent-scouring bath for from 10 to 60 seconds.
5. Process as claimed in claim 1 wherein the textile material remains in an aqueous bath containing the said member for up to 5 minutes.
6. Process as claimed in claim 5 wherein the textile material remains in the aqueous bath for from 2 to 60 seconds.

#### References Cited

##### UNITED STATES PATENTS

|    |           |         |               |       |           |
|----|-----------|---------|---------------|-------|-----------|
| 35 | 2,540,311 | 2/1951  | Wolff         | ----- | 117—138.5 |
|    | 2,729,576 | 1/1956  | Trusler       | ----- | 252—D.C.  |
|    | 3,106,460 | 10/1963 | Topham et al. | ----- | 8—142X    |
|    | 3,404,943 | 10/1968 | Morris        | ----- | 8—139     |

40 MAYER WEINBLATT, Primary Examiner

U.S. CL. X.R.

8—18, 138, 139; 117—137.5

**Disclaimer**

3,575,686.—*John William Case, Norman Frederick Crowder, and Wilfred Arthur Stephen White, Runcorn, England. TREATMENT OF TEXTILES.* Patent dated Apr. 20, 1971. Disclaimer filed Dec. 15, 1969, by the assignee, *Imperial Chemical Industries Limited.*

Hereby disclaims the portion of the term of the patent subsequent to Nov. 4, 1986.

[*Official Gazette September 12, 1972*]